

## UNITED STATES PATENT OFFICE

RUSSELL P. CROTHERS, OF CINCINNATI, OHIO

## PROCESS FOR RECLAIMING ASPHALT FROM RESIDUUM

No Drawing.

Application filed March 27, 1928. Serial No. 265,226.

This invention relates to a process whereby it is possible to reclaim and provide commercial asphalt or pitch from the residuum oils or matter remaining after cracking of petroleum products.

At the present time large masses of residuum products are considered waste at cracking stills. This waste material presents a problem in that it is difficult to dispose of. 10 Heretofore attempts have been made to dispose of this waste matter by burning same, however, it has not been found commercially worth while to use the substance as fuel.

This invention concerns itself with utilizing this waste product to advantage.

The residuum oil obtained from a petroleum cracking still generally contains a very large quantity of free carbon. Free carbon is thoroughly admixed with the asphalt or 20 pitch.

It is an object of this invention to separate the free carbon from the pitch and to then reduce the pitch or asphalt to such state that it is a commercial asphalt.

25 In the ordinary distillation of crude oil the following steps are generally followed:

A given quantity of crude oil is subjected to ordinary distillation for withdrawing various volatile oils such as gasoline. There- 30 after, the resultant mass, comprising kerosene, gas oil, fuel oil and possibly some other substances, is subjected to a cracking process. In carrying on this cracking process the substance is introduced into a so-called crack- 35 ing still and the temperature thereof is raised to a high degree. The cracking process may be carried on in any of the manners commonly employed, however, the result is invariably the same, namely, that there remains a con- 40 siderable quantity of residuum oil that may be withdrawn from the still while in a hot or molten state. There also remains on the bottom of the still a quantity of carbon known as coke. My discovery begins here.

45 The residuum oil is admixed with a quantity of fuel oil and same are caused to flux. Thereafter, the free carbon is separated out or precipitated in any suitable manner, for example, by raising the temperature of the mass to such a degree that the mass remains

in a fluid condition, however, obviating any appreciable disturbance of the mass whereby the free carbon may precipitate and the fluid mass be withdrawn or run from the top of the device in which the process is being carried on. If desired the free carbon may be precipitated or separated from the remainder of the heated substance by means of centrifugal action. Any suitable device may be employed for applying centrifugal force to a mass of residuum product while in a molten state, the free carbon being thrown outwardly and the fluid asphalt or pitch being withdrawn from the center of the device.

The withdrawn asphalt is subsequently 65 treated, preferably by heating, in order to reduce same to commercial asphalt.

The following steps and proportions will give good results:

500 grams of residuum oil is heated to approximately 340 degrees F. 400 grams of fuel oil of a Baumé gravity of about 14 is heated to approximately 200 degrees F. The heated fuel oil is admixed with the residuum and this mixture is stirred and the temperature of the entire mass is raised to about 340 degrees F. Thereupon the substances flux and the temperature of the flowing substance is raised as quickly as possible, to 540 degrees F. The mass is held at temperature of about 540 degrees F. for about forty-five minutes without agitating same. The bulk of the free carbon cakes on the bottom and the asphaltic oil (mass A) is poured off. Thereupon heat is again applied for about ten 75 minutes to the caked carbon and any additional asphaltic oil (mass B) driven out of the carbon is withdrawn. The mass of asphaltic oil (A plus B) is then reheated, as quickly as possible, to about 540 degrees F., 80 and held at that temperature for about twenty-five minutes. A shiny mass develops in the batch. Thereafter the batch is permitted to cool to about 340 degrees F., thereby 85 causing the shiny mass (presumably high melting point, partially decomposed asphalt) to solidify sufficiently to permit withdrawal of the fluid asphalt or asphaltic oil (mass C) and separating the fluid asphalt from the shiny mass. The asphaltic oil (mass C) is 90 95 100

again reheated to approximately 540 degrees F., and retained at that temperature for about twenty-five minutes. There is during this period a precipitation of a small quantity of free carbon (granulated mass). The asphaltic oil (mass D) is poured off and this withdrawn mass is substantially carbon free asphaltic oil and fuel oil. This mass (D) is then reduced in any of the commonly employed processes for obtaining asphalt from crude petroleum. During this period of treatment or distillation the lighter oil, including the fuel oil is distilled off and may be reclaimed and is usable as fuel oil.

15 Although it is practically and commercially desirable to raise the temperatures of the various masses in a minimum of time, it is not essential that the temperatures be raised quickly, although it is wasteful and slows down the production, not to raise the temperatures quickly. Except during the period of fluxing of the fuel oil and residuum oil, there should be as little agitation as possible, in order that the free carbons, when released 20 from union with the pitch or asphalt, may be settled out or precipitated in a minimum of time. The temperatures given are not absolute, although excellent results are attained therefrom. It is desirable that the 25 temperature should not exceed 600 degrees F. at any stage of the process.

From an initial charge of 500 grams of residuum oil and 400 grams of fuel oil, approximately 538.15 grams of commercial asphaltic oil may be reclaimed.

Although the invention is disclosed herein as relating principally to the treatment of residuum oils or products, it is readily obvious that the process may be employed for 40 removing the carbon created during any cracking process of the petroleum. The process may be employed upon fuel oil, whereby to remove the carbon, whereby the value of such fuel oil as a fuel is enhanced, or the 45 treated fuel oil may be reduced to any extent, for example, to commercial asphalt.

What is claimed is:

1. The process of reclaiming asphalt from asphaltic residuum oil, comprising heating a 50 mass of such petroleum residuum oil, adding thereto a quantity of heated fuel oil, heating and admixing the residuum oil and fuel oil until they flux, permitting the free carbon to settle out of the fluxed mass, withdrawing 55 the mass from the precipitated carbon, re-heating and cooling the withdrawn mass and settling out more free carbon and high melting point asphalt, withdrawing the mass from such last settled out substances and reducing the last withdrawn mass to the desired consistency.

2. The process of treating petroleum residuum oil containing asphalt, comprising heating a mass of residuum oil to approximately 60 340 degrees F., adding thereto a quan-

70 tity of fuel oil heated to approximately 200 degrees F., heating and admixing the residuum oil and fuel oil for fluxing same and continuing the heating and admixing until the temperature of that mass is approximately 75 340 degrees F., retaining the temperature of the mass at approximately 340 degrees F., until the substances have completely fluxed; raising the temperature of the fluxed mass to approximately 540 degrees F., maintaining 80 the temperature of the mass at approximately 540 degrees F., for a sufficient period of time to permit settling out or precipitation of free carbon, withdrawing the asphaltic oil from the precipitated carbon; heating the withdrawn asphaltic oil to about 540 degrees F., and maintaining same at that temperature for separating high melting point matter, 85 cooling the mass to approximately 340 degrees F., to permit congealing or coagulation of the high melting point matter and withdrawing of the asphaltic oil, reheating the asphaltic oil to approximately 540 degrees F., to precipitate any additional free carbon 90 remaining therein and then reducing the remaining asphaltic oil into commercial asphalt.

3. The process of treating petroleum residuum oil containing asphalt, comprising the admixing of approximately five parts of residuum oil at approximately 340 degrees F., and four parts of approximately fourteen Baumé gravity fuel oil at approximately 200 degrees F., heating the admixture for attaining fluxing thereof, modifying the temperature of the fluxed mass for separating free carbon and high melting point matter from the asphaltic oil, and reducing the asphaltic oil to commercial asphalt.

In testimony whereof, I have hereunto subscribed my name this 26th day of March, 1928.

RUSSELL P. CROTHERS.

110

115

120

125

130